

## UNITED STATES PATENT OFFICE.

PAUL KEMP AND THEODOR KITTL, OF VIENNA, AUSTRIA.

## BEARING METAL.

No Drawing. Application filed August 10, 1925, Serial No. 49,450, and in Austria August 23, 1924.

This invention relates to alloys of the ternary system lead-tin-antimony containing a high percentage of lead and a considerably smaller amount of tin, which alloys show

5 qualities as suitable for use as bearing metals just as good as alloys containing a high percentage of tin.

For obtaining such result trials have already been made for preventing segregation 10 and increasing the hardness by adding a few per cent of copper to alloys showing approximately the composition: 80% lead, 10% antimony, 5% tin. Furthermore it has been proposed to improve alloys containing 15 a high percentage of lead, with about 15 to 25% of antimony and about 3 to 6% of tin, by adding simultaneously about 1 to 3% of nickel and 0.6 to 1.5% of copper. Adding to such alloys, both nickel and copper, in 20 the ratio stated is claimed to give the surprising effect ameliorating alloys poor in tin to such degree, as to render them equivalent to alloys with high tin contents. It has been proposed also to add insignificant quantities 25 of phosphorus or arsenic (with the nickel and copper), added for augmenting to a small degree the hardness of the resulting alloy. For this purpose it has been proposed to add the 0.6 to 1.5% of copper in 30 the form of phosphor-copper (of which 0.8 to 2.2% were added) or else, to replace the phosphorus totally or partly by arsenic, which was regarded as an equivalent of phosphorus.

35 The present invention is based on the knowledge gained in the course of exhaustive experiments, that alloys of the ternary system lead-tin-antimony with high contents of lead and a low percentage of tin can 40 be made equivalent in respect of all the essential properties, to bearing metals of said ternary system with a high tin contents by adding appropriate quantities of arsenic only without addition of other metals. According 45 to the invention, for bearing metals containing about 65 to 77% of lead, 3 to 14% of tin and 10 to 27% of antimony the quantity of arsenic to be added amounts to from 0.7 to 2.5%.

50 The effect resulting from the addition of arsenic is based on two distinguished proceedings, which both must co-act and which cannot be provoked by the addition of phosphorus. The said two proceedings are the following:

1. Arsenic forms with lead and antimony a ternary eutectic, which is considerably harder than the binary eutectic lead-antimony.

2. Arsenic forms with tin a hard tin-arsenic compound, the composition of which is most likely  $\text{Sn}_3\text{As}_2$ .

From these two facts a very considerable increase of hardness and compressive strength of the alloys results. Moreover 65 the latter also answer in respect of upsetting capability and sliding qualities all the requirements demanded from bearing metals with high tin contents.

In the journal "Metallurgie" of Borchers 70 and Wüst, 1912, page 423, table I, amongst a great number of summarily enumerated lead-antimony-tin alloys also an alloy containing 0.5% of arsenic is indicated, but there is no indication whatever, from which 75 the essential importance of limited arsenic contents of the alloys in question could be derived. In fact, the amount of 0.5%, as indicated there, is too small for producing a substantial amelioration of the alloy, as the 80 tin-arsenic compound, the essential agent which brings about the amelioration of the bearing metal, is not formed to a sufficient extent. Moreover, arsenic containing bearing metals are also mentioned in the journal "Zeitschrift für Metallkunde", 1923, Tome 15, pages 165 and 166, particularly in the table page 165. These alloys however, 85 do not contain any tin, whilst according to the present invention a certain although 90 small amount of tin is indispensable, as the essential condition for the amelioration of the main alloy consists of the formation of the above mentioned tin-arsenic compound.

As this tin-arsenic compound must be 95 present in the alloy in not too small an amount, if a substantial influence on the qualities of the bearing metal ought to be obtained, the contents of arsenic must not go below a certain limit. The lower limit has 100 been stated to be at about 0.7%.

As examples of carrying the invention into practice the following compositions may be given:

1. 5% tin, 25% antimony, 1 to 2% arsenic, 105 the remainder lead. This alloy has a compressive strength of 1650 to 1700 kilogrammes per square centimetre, an upsetting capability of 25% and a hardness of 31 to 33 degrees Brinell.

2. 12% tin, 10% antimony, 2% arsenic, the remainder lead. The compressive strength of this alloy is about the same as that of the alloy according to Example 1, but upsetting capability and hardness are a little less (hardness about 29 degrees Brinell).

As an essential advantage of these alloys in comparison with known alloys having similar percentages of tin, antimony and lead it is to be pointed out, that by the omission of copper as a constituent of the alloy the noxious action of the copper-antimony compounds, is excluded, which particularly in lead alloys exercises an unfavourable effect. If the hardening is effected by the addition of nickel, the upsetting capability of the alloy is considerably diminished and its melting zone is enlarged, owing to the high melting point of nickel. For this reason, when employing bearing metals with nickel contents certain prescriptions for casting are to be closely observed, as otherwise strong segregation would occur and the effective constituent, the nickel, should be

eliminated in the form of difficultly fusible sweepings.

The alloys made according to the present invention are exempt of these drawbacks, but on the other hand show all the advantages of bearing metals with high tin contents. Moreover the alloys made according to Example 2, owing to their nearly eutectic composition, have a very narrow melting zone and in general a particularly low melting temperature, they can therefore be handled very easily and require no special cautions for casting.

We claim:

1. Bearing metals consisting of 65-77% lead, 3-14% tin, 10-27% antimony and 0.7 to 40 2.5% arsenic.

2. Bearing metal consisting of 68 to 69% lead, 5% tin, 25% antimony, and 1-2% of arsenic.

In testimony whereof we have affixed our signatures.

PAUL KEMP.  
THEODOR KITTL.